

H. L. SULMAN & H. F. K. PICARD,  
EXTRACTION OF ZINC,  
APPLICATION FILED JAN. 20, 1917

1,295,080.

Patented Feb. 18, 1919.



Inventors:  
H. L. Sulman &  
H. F. K. Picard,  
by Wilkinson, Gush & Mackay,  
Attorneys.

# UNITED STATES PATENT OFFICE.

HENRY LIVINGSTONE SULMAN AND HUGH FITZALIS KIRKPATRICK PICARD, OF LONDON, ENGLAND, ASSIGNEES TO THE METALS EXTRACTION CORPORATION LIMITED, OF LONDON, ENGLAND.

## EXTRACTION OF ZINC.

1,295,080.

Specification of Letters Patent.

Patented Feb. 18, 1919.

Application filed January 20, 1917. Serial No. 143,448.

To all whom it may concern:

Be it known that we, HENRY LIVINGSTONE SULMAN, a subject of the King of England, and HUGH FITZALIS KIRKPATRICK PICARD, 5 a subject of the King of England, both residing at London, England, have invented certain new and useful Improvements in the Extraction of Zinc, of which the following is a specification.

10 This invention is for improvements in or relating to the extraction of zinc from ores or zinc-containing materials, and it refers more particularly to the preparation of a solution of zinc by dissolving the metal from 15 the ore or other material containing it with an acid. It has for its object to overcome certain difficulties which are met with in carrying out such a process.

It has previously been proposed to treat 20 a zinc ore or zinc-containing material with an acid such as sulfuric acid to dissolve the zinc and form a solution thereof for treatment by electrolysis. In such a process the ore, if a sulfid ore, must be first roasted 25 to convert the sulfid into oxid.

In extracting zinc from an ore or zinc-containing material with acid a difficulty is experienced in completely neutralizing the acid with which the ore is treated, and therefore 30 in fully extracting the zinc from the ore added thereto. For example if a solution containing 10% of acid has zinc oxide in the form of roasted zinc-bearing ore added to it in quantity theoretically sufficient to 35 neutralize all the acid, it is found that complete neutralization is not readily obtained, the last portions of acid remaining unneutralized even after agitation for some time with an excess of roasted ore. In practice the 40 additions of roasted ore to acid solution are made in successive small quantities, with vigorous agitation; but such neutralization is not efficient below 1 or 2% of residual free sulfuric acid, and when approaching this 45 limit it is preferable that the mixture be agitated for longer periods than were necessary for the previous ore additions to the stronger acid solution.

It is also an object of the present invention 50 to overcome this difficulty, and according to this invention the neutralization of the last portions of the acid with which the ore is treated is quickly completed by the addition of zinc hydrate.

One method of carrying this invention into effect will now be described with reference to the accompanying drawing which represents the process diagrammatically for the production of a zinc salt solution for subsequent treatment by electrolysis. A zinc sulfid-containing ore is roasted to convert the zinc into oxid and partially sulfate, and after grinding is added in successive portions to a 10% solution of sulfuric acid. When after such additions in due amounts 55 the liquor is found to contain from 1 to 2% of free acid, the neutralization is completed by the addition of the requisite quantity of zinc hydrate obtained in the manner described below. The mixture is submitted to 60 a short agitation to neutralize completely the acid. Where soluble silica is present the solution is preferably agitated and maintained at a temperature of from 90 to 100° C., so that the soluble silica is caused to be 65 precipitated in a more granular form whereby it is prevented from gelatinizing and from causing trouble in filtration or even the complete jellification of the liquor. The solid material is then separated from the 70 liquor in a filter-press or vacuum or other suitable filtration apparatus, and the clear liquor may be passed over granulated metallic zinc, or preferably agitated with zinc-fume, to remove any copper and cadmium 75 present.

The material left in the filter-press is the undissolved portion of the ore, viz. silica gangue-stuff, insoluble lead and other metallic compounds, ferric oxid, gelatinous 80 silica, etc., but still wetted with some strong zinc sulfate solution.

This is recovered as usual by washing out 85 with water, but the zinc sulfate solution so obtained is necessarily too weak and too voluminous to be added to the main bulk of the filtrate, which in a cyclic electrolytic process, must be kept at the strength and volume suitable for the final electrolytic precipitation of the zinc; from 8% to 10% of 90 zinc as sulfate is a desirable electrolyte. In order to prevent the accumulation of large quantities of these weak liquors and to avoid the necessity of concentrating them and their zinc contents by evaporation, we treat them 95 in a suitable tank or vessel with strong agitation with the requisite quantity of milk of lime, whereby zinc hydrate and calcium

sulfate are precipitated. The pulp is then filtered, the water now free from zinc being run to waste. The precipitate containing zinc hydrate, which is very readily soluble even in dilute acid, thus forms an excellent material for completing the neutralization of an original mixture of ore and acid which cannot, as stated, be completely or efficiently neutralized by roasted ore additions; and is returned to the agitation vessel to complete the neutralization of the acid, in a fresh charge.

The calcium sulfate which accompanies the zinc hydrate is left with the residues in the filtration apparatus on filtration of the neutralized pulp. In this manner the wash waters may be so controlled as to permit the standard volume of liquor, containing all the zinc extracted from the ore, to be returned for electrolytic precipitation.

The zinc sulfate solution, after removal of the copper and cadmium, and iron present is submitted to electrolysis for the separation of the zinc until the solution contains about 10% of sulfuric acid, when it is returned for the treatment of a fresh quantity of roasted ore to neutralize its acid content and replenish its zinc.

Various modifications may be made in the process without departing from this invention. For example, if a carbonate ore is to be treated, it is not necessary to submit it to a preliminary roast before treatment with the acid.

In the following claims the term "zinc-containing material" is to be understood to include zinc ores.

What we claim as our invention and desire to secure by Letters Patent is:—

40 1. In a process for the extraction of zinc from zinc-containing material treating the material with acid to dissolve the zinc, filtering the clear solutions from the residue,

washing the residue to remove the solution remaining therein, adding milk of lime to the said washings to precipitate zinc hydrate and adding the precipitate so obtained to the solution produced from a fresh batch of zinc-containing material by treatment with acid to complete quickly the neutralization of the acid.

2. In a process for the extraction of zinc from zinc-containing material in which the material is treated with an acid, completing the neutralization of the acid by the addition to the solutions of zinc hydrate and agitating the mixture of zinc-containing material residue and neutralized liquor and maintaining it at a temperature of from 90 to 100° C. to cause the gelatinous silica to separate in a more granular form.

3. In a process for the extraction of zinc from zinc-containing material treating the material with acid to dissolve the zinc, adding zinc hydrate to neutralize quickly the remaining acid, agitating the mixture and maintaining it at a temperature of from 90 to 100° C. to cause the gelatinous silica to separate, filtering the clear solutions from the residue, washing the residue to remove the solution remaining therein, adding milk of lime to the said washings to precipitate zinc hydrate and adding the precipitate so obtained to the solution produced from a fresh batch of zinc-containing material by treatment with acid to complete quickly the neutralization of the acid.

In testimony whereof we have signed our names to this specification in the presence of two subscribing witnesses.

HENRY LIVINGSTONE SULMAN.  
HUGH FITZALIS KIRKPATRICK PICARD.

Witnesses:

ALFRED NUTTING,  
HERBERT S. BURSLEY.